

No. 869,012.

PATENTED OCT. 22, 1907.

E. McOUAT & H. W. F. LORENZ.  
FILAMENT FOR INCANDESCENT LAMPS.  
APPLICATION FILED JUNE 29, 1904.

FIG. 1.



FIG. 2.



FIG. 3.



WITNESSES:

*Geo. L. Cheney*  
*F. D. Barnes*

INVENTORS

*Eugene McQuat*  
*Henry W. F. Lorenz*  
BY

*M. M. Mull*  
ATTORNEY

# UNITED STATES PATENT OFFICE.

EUGENE McOUAT AND HENRY W. F. LORENZ, OF AMSTERDAM, NEW YORK.

## FILAMENT FOR INCANDESCENT LAMPS.

No. 869,012.

Specification of Letters Patent.

Patented Oct. 22, 1907.

Application filed June 29, 1904. Serial No. 214,631.

To all whom it may concern:

Be it known that we, EUGENE McOUAT and HENRY W. F. LORENZ, citizens of the United States, and residents of Amsterdam, in the county of Montgomery and State of New York, have invented certain new and useful Improvements in Filaments for Incandescent Lamps, of which the following is a specification.

Our invention relates to plating filaments for incandescent lamps, and the object of our invention is to provide a new process by which said filaments may be plated cheaply, rapidly and effectively.

Reference is to be had to the accompanying drawings which form part of this specification, in which drawings like characters of reference indicate like parts in the several views, and in which

Figure 1 represents a filament which is formed according to our process; Fig. 2 represents a short portion of a filament formed according to our invention, the coating thereof being represented in cross section; 20 this view being upon a much enlarged scale; and Fig. 3 represents in section upon a much enlarged scale a portion of the coating of the carbon core, which is fixed to the core by our process.

We attain our object by the use of the following process: We provide a slightly adhesive liquid or semi-liquid, which is preferably the well-known caramel mixture of water and burnt sugar. To this we add suitable quantities of finely-divided metal in any form, including oxids or nitrids. The mixture is then thoroughly stirred so as to bring the metallic particles into mechanical suspension in the liquid. The filaments to be plated, which are preferably composed of carbon, are then dipped into this mixture, which may be agitated, meanwhile, to maintain a perfect suspension of the metal particles. When the filaments are withdrawn they will be completely covered with a coating composed largely of metallic particles which adhere with the sugary liquid to the body of the filament. The dipped filaments are then subjected to a high heat for the purpose of baking or solidifying the adhering semi-liquid coat.

The baking is preferably effected in a vacuum, or partial vacuum, or in an indifferent gas, so as to prevent the oxygen of the air from acting upon the ingredients composing the coating of the filaments.

In cases where metals are used in the mixture, the filaments may be flashed in the usual manner. The baking process, chars the caramel, and the charred particles are afterward converted into pure carbon

when the filaments are flashed or heated to a higher 50 temperature. The carbon particles of the caramel solution after being carbonized unite to the carbon filament and bind the metal particles to the carbon core, thus forming a complete homogeneous coating on the carbon core. By this process the metal particles 55 constituting the plating are cemented together by particles of carbonaceous matter and adhere to the carbon core of the filament to form a continuous uninterrupted enveloping coat.

A filament made according to our invention and presenting substantially the appearance of an ordinary incandescent filament, is illustrated in Fig. 1. In Fig. 2, 1 represents the carbon core of the filament. In the completed filament this core is enveloped in a coating 2 of the carbonized sugar of the binder, and 60 this coating 2 is surrounded and enveloped in a second coating 3, which consists in the finely divided particles of metal cemented together by the carbonized sugar which is located in the interstices between the particles. The carbon coat 2 occurs by reason of the 65 fact that the particles of metal will not adhere directly to the core 1, but will adhere to the outer side of the coat of carbonized sugar. The carbonized sugar, of course, adheres tightly to the carbon core, and in this way a very compact and serviceable filament is produced. In Fig. 3 the small metal particles 4 are represented as highly magnified, the same being securely cemented together by the carbonized sugar 5 deposited 70 in the interstices therebetween.

All metals can be applied as suggested by applicants' 80 method but only such as are of a suitably high melting answer the purpose well. A partial list of such metals includes titanium, tungsten, molybdenum, uranium, thorium, tantalum, vanadium, columbium, chromium, manganese, cobalt and nickel.

Having thus described our invention, we claim as new and desire to secure by Letters Patent:

The process of making incandescent filaments, which consists in dipping a carbonized core in a caramel solution containing finely divided metallic light-emitting particles in mechanical suspension whereby a coat is deposited on said core through which said particles are dispersed, and carbonizing said coat to render said coat and said particles integral with said core.

Signed at Albany, N. Y. this 25th day of June 1904.

EUGENE McOUAT.  
HENRY W. F. LORENZ.

Witnesses:

WALTER E. WARD.  
FRANKLIN HAVENS.